

# UNITED STATES PATENT OFFICE.

EMILE BRONNERT, OF MÜLHAUSEN, ALSACE-LORRAINE, FRANCE.

## MANUFACTURE OF VISCOSE SILK.

1,393,198.

Specification of Letters Patent. Patented Oct. 11, 1921.

No Drawing.

Application filed August 30, 1920. Serial No. 406,911.

To all whom it may concern:

Be it known that I, EMILE BRONNERT, a citizen of the Republic of France, residing at 1 Quai du Barrage, in Mülhausen, Alsace-Lorraine, France, have invented certain new and useful Improvements in the Manufacture of Viscose Silk, (for which I have filed application in Germany, filed January 23, 1919; Belgium, Denmark, England, Finland, France, Netherlands, Italy, Norway, Austria, Sweden, Switzerland, Spain, Czechoslovakia, Hungary, filed March 22, 1920; and Poland, filed April 26, 1920,) of which the following is a specification.

15 This invention relates to a process for the manufacture of very fine threads of viscose silk by precipitation of raw viscose solutions by means of an acid.

It is well known that in the production of 20 artificial silk threads from viscose, by means of mineral acid, there must correspond to every age of the viscose a definite acid concentration with a definite spinning length and bath temperature.

25 These observations related at the time to the usual commercial class of silk of about 7-8 deniers.

Now by means of experiments applicant has found that the degree of fineness of the 30 produced thread is a function of the acid concentration, either possibly because the acid is bound to a base that can be driven out by soda lye, or because it is only partially bound or partly free.

35 Trials with pure acid (sulfuric acid, hydrochloric acid, etc.), or with acid that only contains so much salt as to be equal to that which is unavoidably formed by spinning, have given the astonishing result 40 that the conditions here are similar to these prevailing with the use of acid baths containing much salt.

Furthermore there is also the astonishing fact that, in order to obtain the maximum degree of fineness, acid concentrations can and must be employed which have hitherto been regarded as directly harmful to the tenacity or strength of the threads especially when working with an increased temperature.

50 Upon the basis of numerous experiments applicant has found that, on spinning by means of the usual apparatus and with the

nozzle openings of 0.1 mm. used heretofore for the usual artificial silk threads of about 7.5 deniers, threads of any degree of fineness desired can be made when, under observance of the same drawing off speed and of the feed quantity of viscose solution corresponding to the deniers required at the time, the concentration of the acid is so selected that the minimum concentration of the acid, which gives a faultless spinning with a coarser denier must for a further desired concentration be chosen approximately inversely proportionated to the square roots of the two thread denier figure.

This law, occurring in using acid alone, is drawn from the following practical examples:

1. Raw viscose of about 8 degrees of ripeness (chlorid of ammonia) is spun in the usual manner with a correspondingly regulated feed of the viscose, for example in sulfuric acid of about 250 gr. per liter; threads of 2 deniers which can easily be wound up being obtained.

2. Raw viscose of about 7 degrees of ripeness (chlorid of ammonium) is spun in the usual manner with a correspondingly regulated feed of the viscose, for instance in sulfuric acid of about 350 gr. per liter, threads of about 1 denier being obtained which can be readily wound up.

As a matter of fact, according to the above mentioned example the concentration of the second bath must be calculated according to the formula

$$\frac{x}{250} \pm \frac{\sqrt{2}}{\sqrt{1}}$$

90

or

$$x = 250 \cdot \sqrt{2} = 354$$

or approximately 350 gr., as stated in the second example.

From the foregoing examples, it will be seen that the acid concentrations of two coagulating baths are to each other, inversely as the square roots of the fineness of the threads produced in said baths under similar conditions, measured in denier numbers. Or, differently stated, the relative fineness of the threads produced from two acid coagulating baths under similar conditions, measured in denier numbers, are to each other,

inversely as the squares of the acid concentrations of the baths.

Symbolically represented, we have

$$5 \quad \frac{C_1}{C_2} = \frac{\sqrt{D_2}}{\sqrt{D_1}}$$

and by squaring both sides of the equation we get

$$10 \quad \frac{D_2}{D_1} = \frac{C_1^2}{C_2^2} \text{ or } \frac{D_1}{D_2} = \frac{C_2^2}{C_1^2}$$

where  $C_1$  = acid concentration of first bath.

$C_2$  = acid concentration of second bath.

15  $D_1$  = fineness of thread produced in  $C_1$  measured in deniers.

$D_2$  = fineness of thread produced in  $C_2$  measured in deniers.

I claim:

20 1. The process of producing artificial silk threads comprising forcing viscose through suitable openings into a coagulating bath consisting of an acid, the concentration of which is proportional to the fineness of the 25 thread desired.

2. The process of producing artificial silk threads comprising forcing viscose through

suitable openings into a coagulating bath consisting of an acid, the concentration of which is inversely proportional to the square root of the fineness of the thread desired, measured in deniers.

3. In the process of producing artificial silk threads by forcing viscose through suitable openings into a coagulating acid bath, 30 the method of predetermining the acid concentration necessary to produce a thread of a given fineness, which consists in first determining the minimum concentration of the acid which gives a faultless spinning thread 40 of a certain fineness and then varying the concentration of the bath in accordance with the equation

$$\frac{C_1}{C_2} = \frac{\sqrt{D_2}}{\sqrt{D_1}}$$

45

In witness whereof, I have hereunto signed my name in the presence of two subscribing witnesses.

EMILE BRONNERT.

Witnesses:

L. R. DE SALIS,  
N. L. MEINEBERGER.